# EUROPEAN PATENT SPECIFICATION

(11) **EP 3 590 628 B1**
(45) Date of publication and mention of the grant of the patent: **18.05.2022**
(21) Application number: 18760588.6
(22) Date of filing: 02.03.2018
(51) Int. Cl.: B22D 41/50, B22D 11/115

(54) **CONTINUOUS CASTING METHOD**
STRANGGIESSVERFAHREN
PROCÉDÉ DE COULÉE CONTINUE

(30) Priority: 03.03.2017 JP 2017040658; 04.07.2017 WO PCT/JP2017/024528
(43) Date of publication of application: 08.01.2020
(73) Proprietor: Nippon Steel Stainless Steel Corporation, Chiyoda-ku Tokyo 1000005 (JP)
(72) Inventor: HONDA, Yuki, Tokyo 100-8366 (JP); MORIKAWA, Hiroshi, Shunan-shi Yamaguchi 746-0023 (JP); SUZUKI, Yasuhiro, Tokyo 100-8366 (JP)
(74) Representative: Clarke Modet & Co.
(86) International application number: PCT/JP2018/008066
(87) International publication number: WO 2018/159821

(56) References cited:
- EP-A1- 2 038 081
- EP-A1- 2 092 998
- EP-A1- 2 151 291
- WO-A1-2004/050277
- JP-A- H10 166 120
- JP-A- S50 145 324
- JP-A- 2000 280 050
- JP-A- 2007 319 923
- JP-A- 2008 137 056
- JP-A- 2010 029 936
- JP-A- 2016 022 493
- JP-B1- 6 129 435
- JP-B2- 3 817 209
- JP-B2- 5 791 234
- US-A- 4 042 007

## Description

### Technical Field

The present invention relates to a method for continuously casting steel while carrying out electromagnetic stirring.

### Background Art

In continuous casting of steel, there is a problem that a foreign matter, such as an air bubble and an oxide, which is inevitably incorporated into molten steel in a mold is captured into a solidified shell and, consequently, a defect (flaw) is formed on a surface of a steel sheet (slab) obtained through a hot rolling step or a cool rolling step. As a solution to the problem, electromagnetic stirring is widely employed. By the electromagnetic stirring, a flow of the molten steel in the mold is controlled so that the foreign matter in the molten steel is floated and is then captured by a mold powder applied to a surface of the molten steel. Patent Literature 1 discloses an example of such a method.

In the technique disclosed in Patent Literature 1, a submerged nozzle is used which has two discharge holes through each of which molten metal is discharged upward at an angle of 5° to 30°. Through the two discharge holes, the molten metal is discharged toward short sides of a mold. Then, by electromagnetic stirring, a driving force acting in a direction perpendicular to a casting direction is applied to the molten metal in a vicinity of a meniscus near each of two long-side surfaces of the mold. With this configuration, a temperature of the molten metal in a vicinity of its surface is kept high, and a flow of the molten metal, which flow is uniform and perpendicular to the casting direction, is formed.

### Citation List

### [Patent Literature]

[Patent Literature 1] Japanese Patent Application Publication Tokukaihei No. 10-166120 (Published on June 23, 1998).
[Patent Literature 2] European Patent application EP 2 092 998 A1 of NIPPON STEEL CORP (Published on August 26, 2009).
[Patent Literature 3] Document JP 3 817 209 B2 of NIPPON STEEL CORP (Published on September 6, 2006).
[Patent Literature 4] Document US 4 042 007 A of ZAVARAS ALEXANDER A ET AL (Published on August 16, 1977).
[Patent Literature 5] Document JP 2007 319 923 A of NIPPON STEEL CORP (Published on December 13, 2007)
[Patent Literature 6] Document EP 2 038 081 A1 of ABB AB (Published on March 25, 2009)
[Patent Literature 7] Document JP 2016 022 493 A of NIPPON STEEL & SUMITOMO METAL CORP (Published on February 8, 2016)
[Patent Literature 8] Document JP 5 791 234 B2 of JFE STEEL CORP (Published on October 7, 2015
[Patent Literature 9] Document WO2004/050277 A1 of ABB AB and KOLLBERG STEN ET AL (Published on June 17, 2004)
[Patent Literature 10] Document EP 2 151 291 A1 of SUMITOMO METAL IND of February 10, 2010.
[Patent Literature 11] Document JP 2010 029 936 A of JFE STEEL CORP of February 12, 2010.

### Summary of Invention

### Technical Problem

However, Patent Literature 1 does not clearly disclose a method of forming a stirring flow for increasing cleaning of a foreign matter from the molten metal. Thus, the technique disclosed in Patent Literature 1 has a problem that an effect of suppressing capture of a foreign matter into a solidified shell is not sufficient.

An object of an aspect of the present invention is to effectively suppress capture of a foreign matter into a solidified shell.

### Solution to Problem

The scope of the present invention is defined by independent claim 1, and further embodiments of the invention are specified in dependent claims 2-4.

### Advantageous Effects of Invention

According to an aspect of the present invention, it is possible to effectively suppress capture of a foreign matter into a solidified shell.

### Brief Description of Drawings

Fig. 1 is a schematic view illustrating a configuration of a continuous casting device which is not part of the present invention.
Fig. 2 is a cross-sectional view of the continuous casting device, obtained by cutting the continuous casting device along a horizontal plane at a height of a surface of molten steel in a mold included in the continuous casting device.
Fig. 3 is a cross-sectional view of a vicinity of the surface of the molten steel in the continuous casting device, obtained by cutting the continuous casting device along a plane which passes through a center of the mold and which is parallel to long-side molds included in the mold.
Fig. 4 is a cross-sectional view of the vicinity of the surface of the molten steel in the continuous casting device, obtained by cutting the continuous casting device along a plane which passes through the center of the mold and which is parallel to short-side molds included in the mold.
Fig. 5 is a cross-sectional view of a continuous casting device which is not part of the present invention, and is a cross-sectional view of a vicinity of a surface of molten steel in the continuous casting device, obtained by cutting the continuous casting device along a plane which passes through a center of a mold included in the continuous casting device and which is parallel to long-side molds included in the mold.
Fig. 6 shows the numbers of macro-streak-flaws per square millimeter on each of an example strand of the present invention and a comparative example strand. (a) of Fig. 6 is a graph showing the numbers of macro-streak-flaws present at a location 2 mm below a surface layer. (b) of Fig. 6 is a graph showing the numbers of macro-streak-flaws present at a location 3 mm below the surface layer.

### Description of Embodiments

The following description will discuss a continuous casting method in accordance with Embodiment 1 of the present invention with reference to Figs. 1 through 4. As used herein, an expression "A to B" means "not less than A and not more than B".

Fig. 1 is a schematic view illustrating a configuration of the continuous casting device 1A which is not part of the invention. As illustrated in Fig. 1, the continuous casting device 1A includes a ladle 2, a tundish 3, a mold 10, a submerged nozzle (discharge nozzle) 40A, and electromagnetic stirring devices (stirring devices) 50A and 50B. The ladle 2 receives molten steel supplied from a steel converter.

The tundish 3 is a member for storing the molten steel transferred from the ladle 2 and removing a foreign matter such as an oxide. The molten steel stored in the tundish 3 is transferred into the mold 10 through the submerged nozzle 40A (later described).

The mold 10 is a mold for cooling the molten steel thus transferred so that a solidified shell C is formed against an inner surface of the mold 10. The solidified shell C is sent out from a bottom of the mold 10. Fig. 2 is a cross-sectional view of the continuous casting device 1A, obtained by cutting the continuous casting device 1A along a horizontal plane at a height of a surface S of molten steel in the mold 10. As illustrated in Fig. 2, a contour shape of the inner surface of the mold 10 cut at the horizontal plane is a rectangular shape. The mold 10 includes (i) long-side molds 11A and 11B facing each other and (ii) short-side molds 12A and 12B facing each other. The long-side molds 11A and 11B have long-side surfaces (first surface) 11Aa and 11Ba, respectively, which form the inner surface of the mold 10. The short-side molds 12A and 12B have short-side surfaces (second surface) 12Aa and 12Ba, respectively, which form the inner surface of the mold 10. In other words, the long-side surfaces 11Aa and 11Ba and the short-side surfaces 12Aa and 12Ba which intersect the long-side surfaces 11Aa and 11Ba form a surrounding structure. Hereinafter, a horizontal direction which is parallel to the long-side molds 11A and 11B will be referred to as a "long-side direction LD", and the horizontal direction which is parallel to the short-side molds 12A and 12B will be referred to as a "short-side direction SD" (see Fig. 2).

The submerged nozzle 40A is a member for transferring, into the mold 10, the molten steel stored in the tundish 3. The submerged nozzle 40A is provided so that an upper end of the submerged nozzle 40A is connected to the tundish 3 and a lower end of the submerged nozzle 40A is located substantially at a center of the mold 10 (that is, in Fig. 2, substantially at a center of the rectangular shape formed by the long-side surfaces 11Aa and 11Ba and the short-side surfaces 12Aa and 12Ba).

Fig. 3 is a cross-sectional view of a vicinity of the surface S in the continuous casting device 1A, obtained by cutting the continuous casting device 1A along a plane which passes through the center of the mold 10 and which is parallel to the long-side molds 11A and 11B of the mold 10. Note that, since the continuous casting device 1A has a structure symmetrical about the submerged nozzle 40A, Fig. 3 illustrates a region which includes the submerged nozzle 40A and the short-side mold 12B, in a state where the region is enlarged. The submerged nozzle 40A has two discharge holes 41A, as illustrated in Fig. 3. The two discharge holes 41A are each located inside the mold 10, and are each a hole for discharging the molten steel which has been supplied from tundish 3 and which has passed through an inside of the submerged nozzle 40A. The two discharge holes 41A are formed on respective sides of the submerged nozzle 40A which sides are located in the long-side direction LD. Through the two discharge holes 41A, the molten steel is discharged in directions each parallel to the long-side surfaces 11Aa and 11Ba. Each of the two discharge holes 41A is formed so that a discharge direction 60 of a discharge flow is directed upward with respect to the horizontal plane. Hereinafter, an angle formed by the discharge direction 60 of each of the two discharge holes 41A and the horizontal plane will be referred to as a discharge angle θ.

According to the continuous casting device 1A, the molten steel is continuously supplied to the mold 10 through the two discharge holes 41A of the submerged nozzle 40A, and the surface S (also referred to as a meniscus) of the molten steel is formed at a given height inside the mold 10. Note that, although the surface S swings to an extent during continuous casting, an average height of the surface S is regarded as a location of the surface S in the present specification. Note also that a mold powder (not illustrated) for capturing a foreign matter such as an air bubble and an oxide is applied to the surface S.

The electromagnetic stirring devices 50A and 50B are devices for causing, by electromagnetic forces, a stirring flow (swirling flow) with respect to the molten steel in the vicinity of the surface S in the mold 10. Fig. 4 is a cross-sectional view of a vicinity of the surface S in the continuous casting device 1A, obtained by cutting the continuous casting device 1A along a plane which passes through the center of the mold 10 and which is parallel to the short-side molds 12A and 12B of the mold 10. The electromagnetic stirring devices 50A and 50B are provided on back surfaces of the long-side molds 11A and 11B, respectively, as illustrated in Fig. 4. The electromagnetic stirring devices 50A and 50B include stirring coil cores 51A and 51B, respectively. Each of the stirring coil cores 51A and 51B applies an electromagnetic force to the molten steel in the mold 10, at a height at which the each of the stirring coil cores 51A and 51B is provided. Specifically, the stirring coil core 51 A of the electromagnetic stirring device 50A applies, to the molten steel in a vicinity of the long-side mold 11A, an electromagnetic force parallel to the long-side direction LD. Similarly, the stirring coil core 51B of the electromagnetic stirring device 50B applies, to the molten steel in a vicinity of the long-side mold 11B, an electromagnetic force parallel to the long-side direction LD. Note, however, that the continuous casting device 1A is configured such that a direction of the electromagnetic force applied to the molten steel by the stirring coil core 51A and a direction of the electromagnetic force applied to the molten steel by the stirring coil core 51B are opposite to each other. This causes a stirring flow to be formed in the horizontal direction in the vicinity of the surface S in the mold 10 (see an black arrows in Fig. 2). In Embodiment 1, the electromagnetic stirring devices 50A and 50B are provided so that respective upper ends of the stirring coil cores 51A and 51B are each located a given distance below the surface S.

In Fig. 4, a region A1 indicates a region between an upper end and a lower end of each of the two discharge holes 41A, which upper end and lower end are located in a vertical direction. As illustrated in Fig. 4, the stirring coil cores 51A and 51B are provided so as to include, in the vertical direction, the whole two discharge holes 41A. With this configuration, electromagnetic forces are applied, by the stirring coil cores 51A and 51B, to the molten steel discharged through the two discharge holes 41A from a time point when the molten steel is discharged.

The electromagnetic stirring devices 50A and 50B cause a stirring flow with respect to the molten steel in the mold 10. Note, here, that the stirring flow is not formed only in a region located at the height at which each of the stirring coil cores 51A and 51B is provided. That is, in a case where a stirring flow is caused in a region A2 in which the stirring coil cores 51A and 51B are provided, the molten steel, present in regions each extending upward or downward from the region A2 by a certain distance, is also caused to swirl in the mold 10, so that a stirring flow is caused. In the present specification, a region including the region A2 and the "regions each extending upward or downward from the region A2 by a certain distance" will be referred to as a stirring region A3 which is formed by the electromagnetic stirring devices 50A and 50B (see Fig. 4). Specifically, the stirring region A3 in the present specification means a region in which a flow velocity of the molten steel falls within a range of 0.20 m/s to 0.40 m/s. It known that, in a case where a flow velocity of molten steel in a vicinity of a surface S falls within a range of 0.20 m/s to 0.40 m/s, it is possible to reduce both a surface defect and an internal defect of steel to be produced. According to the continuous casting device 1A in accordance with Embodiment 1, the stirring coil cores 51A and 51B are provided so that the stirring region A3 includes the surface S.

Note that the continuous casting device 1A is configured such that the electromagnetic stirring devices 50A and 50B are provided so that the respective upper ends of the stirring coil cores 51A and 51B are each located the given distance below the surface S. However, the continuous casting device which is not part of the present invention is not limited to such a configuration, and can be alternatively configured such that the respective upper ends of the stirring coil cores 51A and 51B are each located at a height corresponding to the height of the surface S or each located above the surface S. Also in such cases, it is possible to configure the continuous casting device so that the stirring region includes the surface S.

The continuous casting device 1A in accordance with Embodiment 1 is configured as follows. That is, a substantially whole amount of the molten steel discharged through each of the two discharge holes 41A of the submerged nozzle 40A is caused to reach the surface S, by appropriately setting the discharge angle θ, a distance L between (i) a center of each of the two discharge holes 41A and (ii) the surface S, and a distance W between the short-side molds 12A and 12B (that is, a length of each of the long-side surfaces 11Aa and 11Ba in the horizontal direction).

Here, the following description will discuss, with reference to Fig. 3, a "reached location" on the surface S which location is reached by the discharge flow caused by the molten steel discharged through a discharge hole 41A. As illustrated in Fig. 3, a center of an opening of the discharge hole 41A is regarded as a starting point, and a point at which the surface S intersects a half line extending in the discharge direction 60 from the starting point is regarded as a point P. In other words, the point P is a point on the surface S which point is reached by the molten steel, discharged through the discharge hole 41A, in a case where the molten steel discharged through the discharge hole 41A proceeds straight. The discharge flow from the discharge hole 41A proceeds through the molten steel in the mold 10 while spreading to some extent. By setting a discharge velocity, at which the molten steel is discharged through the discharge hole 41A, so as to be higher than a given velocity, it is possible to cause the substantially whole amount of the molten steel discharged through the discharge hole 41A to directly reach the point P and the surface S in a vicinity of the point P. In Embodiment 1, the point P and the vicinity of the point P will be referred to as a "reached location". In Embodiment 1, the stirring region A3 incudes a whole line segment via which the center of the opening of the discharge hole 41A and the point P are connected to each other.

Note that, in a case where the discharge angle θ is excessively wide or in a case where the distance L is excessively short, the surface S excessively ruffles because the discharge flow from the discharge hole 41A directly reaches the surface S (reached location), so that the mold powder present on the surface S is highly likely to be entrapped in the solidified shell C as a foreign matter. Therefore, the discharge angle θ is not more than 30°. In the present invention, a velocity of the discharge flow is 300 mm/s to 1150 mm/s, and the distance L is not less than 180 mm.

In a case where the distance L is excessively long, time it takes for the discharge flow to reach the surface S (reached location) becomes longer. As a result, time it takes for a high-temperature discharge flow to reach the surface S in a vicinity of each of the short-side molds 12A and 12B becomes longer, and a temperature of the surface S of the molten steel in the vicinity of each of the short-side molds 12A and 12B becomes lower. A decrease in a temperature of the molten steel causes generation of an ununiform initial solidified shell having a hook-like cross section. This ultimately causes an increase in entrapment of a foreign matter into the solidified shell C. Therefore, in the present invention the velocity of the discharge flow is 300 mm/s to 1150 mm/s, and the distance L is not more than 230 mm.

As an example of the configuration of the continuous casting device 1A, in a case where the distance W is longer than 520 mm, it is possible to cause the substantially whole amount of the molten steel discharged through the discharge hole 41A of the submerged nozzle 40A to reach the surface S (reached location), by setting the discharge angle θ to 30° and setting the distance L to 150 mm (for example, setting a width, in an up-and-down direction, of the discharge hole 41A to 58 mm, and setting a distance between the surface S and an upper end of the discharge hole 41A to 121 mm).

As has been described, the continuous casting method object of the invention carried out with use of the continuous casting device 1A includes: a discharging step of discharging, through the two discharge holes 41A located in the mold 10, the molten steel upward with respect to the horizontal direction and in the directions parallel to the long-side molds 11A and 11B; and a stirring step of stirring the molten steel so that the stirring region A3 includes a whole line segment via which a center of an opening of each of the two discharge holes 41A and the point P are connected to each other.

With this configuration, it is possible to cause most of high-temperature molten steel discharged through each of the two discharge holes 41A to reach the surface S, and accordingly possible to delay solidification of the molten steel in the vicinity of the surface S. This makes it possible to increase a stirring effect of each of the electromagnetic stirring devices 50A and 50B which stirring effect is brought about in the vicinity of the surface S, and possible to effectively suppress capture of a foreign matter, which is present in the molten steel, into a solidified shell C.

Furthermore, since a distance between each of the two discharge holes 41A and the surface S is short, the discharge flow reaches the surface S before the velocity of the discharge flow decreases. This makes it easy to float a foreign matter, such as an air bubble or an inclusion in the molten steel, by the discharge flow whose velocity is high, and makes it easy to cause the mold powder to capture the foreign matter. Moreover, since the distance between (i) each of the two discharge holes 41A and (ii) the surface S is short, it is possible to suppress diffusion of the discharge flow in a flow path through which the discharge flow reaches the surface S, and accordingly possible to avoid blocking the stirring flow.

The discharge flow having reached the surface S is divided into (i) a flow toward the short-side mold 12A or 12B and (ii) a flow toward the submerged nozzle 40A (that is, the center of the mold 10), as illustrated in Fig. 3. As a result, it is possible to uniform the temperature of the molten steel in the vicinity of the surface S.

### Embodiment 2

The following description will discuss another embodiment which is not part of the present invention with reference to Fig. 5. Note that, for convenience, an identical reference sign will be given to a member having a function identical to that of a member described in the foregoing embodiment.

A continuous casting device 1B in accordance with Embodiment 2 includes a submerged nozzle 40B having a structure different from that of the submerged nozzle 40A in Embodiment 1.

Fig. 5 is a cross-sectional view of a vicinity of a surface S in the continuous casting device 1B, obtained by cutting the continuous casting device 1B along a plane which passes through a center of a mold 10 and which is parallel to long-side molds 11A and 11B of the mold 10.

As illustrated in Fig. 5, the continuous casting device 1B in accordance with Embodiment 2 includes the submerged nozzle 40B instead of the submerged nozzle 40A in Embodiment 1.

The submerged nozzle 40B has two discharge holes 41B (see Fig. 5). Each of the two discharge holes 41B is formed so that a discharge direction 70 of molten steel is directed upward with respect to a horizontal plane. Hereinafter, an angle formed by the discharge direction 70 of each of the two discharge holes 41B and the horizontal plane will be referred to as a discharge angle ϕ.

The continuous casting device 1B in accordance with Embodiment 2 is configured as follows. That is, a substantially whole amount of the molten steel discharged through each of the two discharge holes 41B is caused to reach a corresponding one of short-side molds 12A and 12B (more specifically, a solidified shell C formed against the corresponding one of the short-side molds 12A and 12B), by appropriately setting the discharge angle ϕ, a distance L between (i) a center of each of the two discharge holes 41B and (ii) the surface S, and a distance W, on the surface S, between short-side molds 12A and 12B.

Here, the following description will discuss, with reference to Fig. 5, a "reached location" on each of the short-side molds 12A and 12B which location is reached by a discharge flow caused by the molten steel discharged through a corresponding one of the two discharge holes 41B. As illustrated in Fig. 5, a center of an opening of a discharge hole 41B is regarded as a starting point, and a point at which the short-side mold 12B intersects a half line extending in the discharge direction 70 from the starting point is regarded as a point Q. In other words, the point Q is a point on the short-side mold 12B which point is reached by the molten steel, discharged through the discharge hole 41B, in a case where the molten steel discharged through the discharge hole 41B proceeds straight. The discharge flow caused by the molten steel discharged through the discharge hole 41B proceeds through the molten steel in the mold 10 while spreading to some extent. By setting a discharge velocity at which the molten steel is discharged through the discharge hole 41A so as to be higher than a given velocity, it is possible to cause the substantially whole amount of the molten steel discharged through the discharge hole 41B to directly reach the short-side mold 12B. In Embodiment 2, the point Q and a vicinity of the point Q will be referred to as a "reached location". The point Q is located in the vicinity of the surface S.

In Embodiment 2, the continuous casting device 1B is configured such that a stirring region, formed by electromagnetic stirring devices 50A and 50B, at least includes, in a vertical direction, a region ranging from the "reached location" (the point Q and the vicinity of the point Q) to a lower end of the discharge hole 41B. This causes the stirring region, formed by the electromagnetic stirring devices 50A and 50B, to include a whole line segment via which the center of the opening of the discharge hole 41B and the point Q are connected to each other.

As an example of the configuration of the continuous casting device 1B, in a case where the distance W is 1430 mm to 1650 mm and a velocity of the discharge flow is 300 mm/s to 1150 mm/s, it is possible to cause the substantially whole amount of the molten steel discharged through the discharge hole 41B of the submerged nozzle 40B to reach the "reached location", by setting the discharge angle ϕ to 5° and setting the distance L to 125 mm (for example, setting a width, in an up-and-down direction, of the discharge hole 41B to 50 mm, and setting a distance between the surface S and the discharge hole 41A to 100 mm).

As has been described, a continuous casting method carried out with use of the continuous casting device 1B includes: a discharging step of discharging, through the two discharge holes 41B located in the mold 10, the molten steel upward with respect to a horizontal direction and in directions parallel to long-side molds 11A and 11B; and a stirring step of stirring the molten steel so that the stirring region, formed by the electromagnetic stirring devices 50A and 50B, includes a whole line segment via which a center of an opening of each of the two discharge holes 41B and the point Q are connected to each other.

With this configuration, it is possible to cause most of high-temperature molten steel discharged through each of the two discharge holes 41A to reach the vicinity of the surface S, and accordingly possible to delay solidification of the molten steel in the vicinity of the surface S. This makes it possible to increase a stirring effect of each of the electromagnetic stirring devices 50A and 50B which stirring effect is brought about in the vicinity of the surface S, and possible to effectively suppress capture of a foreign matter, which is present in the molten steel, into a solidified shell C.

Each of the continuous casting devices 1A and 1B has a structure in which the solidified shell C and part of the molten steel are drawn out from a lower end part of the mold 10. Therefore, the discharge flow from each of the two discharge holes 41B receives a downward force. Thus, in a case where the continuous casting device 1B has a narrow discharge angle ϕ, the discharge flow from each of the two discharge holes 41B is likely to proceed outside the stirring region. Accordingly, the molten steel is preferably discharged at an angle of not less than 5°, as the discharge angle ϕ. This allows the stirring region to absolutely include the discharge flow from each of the discharge holes 41B.

### Embodiment 3

In Embodiment 3, preferred setting of an electromagnetic stirring device in continuous casting will be described.

The following shows parameters in continuous casting in Embodiment 3. Note that a term in square brackets indicates a unit.
α: a discharge angle of a discharge hole 41A or a discharge hole 41B [°]
A: a discharge area of the discharge hole 41A or the discharge hole 41B [m2]
W: a casting width [m] (horizontal distance between short-side surfaces 12Aa and 12Ba)
T: a casting thickness [m] (horizontal distance between long-side surfaces 11Aa and 11Ba)
V: a discharge velocity at which molten steel is discharged through the discharge hole 41A or the discharge hole 41B [m/s]
Vc: a casting speed [m/s]
L: a submergence depth to which a submerged nozzle 40A or a submerged nozzle 40B is submerged [m] (distance between a center of the discharge hole 41A or the discharge hole 41B and a surface S)
B: a magnetic flux density at a location in the molten steel, which location is 15 mm apart, in a horizontal direction, from each of the long-side surfaces 11Aa and 11Ba [G]
f: a frequency of an electromagnetic stirring device 50A or an electromagnetic stirring device 50B [Hz]
σ: an electric conductivity of a secondary conductor (the molten steel at 1500°C) [1/µΩ-m]

First, since a volume of the molten steel discharged through the discharge hole 41A or 41B is identical to a volume of cast steel, the following Expression 1 is established.$\left(A\times 2\right) \times V = W \times T \times Vc$

A discharge velocity V is determined in accordance with the following Expression 2 on the basis of Expression 1. $V = W \times T \times Vc/2A$

Therefore, a velocity Vy, in a vertical direction, of the molten steel discharged through the discharge hole 41A or 41B is obtained in accordance with the following Expression 3. $Vy = V \times sin α = W \times T \times Vc \times sin α / 2 A$

Thus, time t it takes for the molten steel to reach the surface S from the discharge hole 41A or 41B (surface reaching time t) is obtained in accordance with the following Expression 4. $t = L/Vy = L \times W \times T \times Vc \times sin α / 2 A$

Stirring hydraulic power H applied to the molten steel is obtained in accordance with the following Expression 5. $H = B2 \times f \times σ$

Therefore, an impulse I which the molten steel, discharged through the discharge hole 41A or 41B, receives by the time when the molten steel reaches the surface S is obtained in accordance with the following Expression 6. $I = H \times t = B2 \times f \times σ \times L \times W \times T \times Vc \times sin α / 2 A$

According to a continuous casting method in accordance with Embodiment 3, it is preferable to set the magnetic flux density B, the frequency f, and the casting speed Vc so that the impulse I is 0.4 × 107 G2/µΩ-m to 2.5 × 107 G2/µΩ-m, in a case where the discharge angle α, the discharge area A, the casting width, the casting thickness T, and the submergence depth L have respective given values. This makes it possible to form a stirring flow which is highly effective in cleaning a foreign matter from the molten steel, even in a case where a kind of the molten steel is changed.

The present invention is not limited to the embodiments, but can be altered by a skilled person in the art within the scope of the claims. The present invention also encompasses, in its technical scope, any embodiment derived by combining technical means disclosed in differing embodiments.

### Example 1

The following description will discuss an Example of the present invention.

In Example 1, continuous casting of SUH409L and SUS439, each of which is a kind of ferrite-based steel, was carried out under the following conditions.

### (Continuous casting conditions)

A discharge angle θ of each discharge hole 41A: 30°

A width, in a vertical direction, of each discharge hole 41A: 58 mm

A distance L, in the vertical direction, between a surface S and a center of each discharge hole 41A: 180 mm

A distance W between short-side molds 12A and 12B: 1042 mm

A casting speed: 1.30 m/min

A discharge velocity: 865 mm/s

A thickness of a strand: 200 mm

A magnetic flux density at a location 15 mm apart, in a thickness direction, from each of long-side surfaces 11Aa and 11Ba: 1150 G

The above conditions are conditions under which, in a case where stirring is carried out with use of electromagnetic stirring devices 50A and 50B, (i) a substantially whole amount of molten steel discharged through each discharge hole 41A directly reaches a surface S and (ii) the molten steel is included in a stirring region, formed by the electromagnetic stirring devices 50A and 50B, until the molten steel reaches the surface S from when the molten steel is discharged through the each discharge hole 41A.

In Example 1, evaluation was carried out with respect to (i) strands prepared while stirring was carried out with use of the electromagnetic stirring devices 50A and 50B (a strand of SUH409L will be referred to as an example strand 1, and a strand of SUS439 will be referred to as an example strand 2) and (ii) strands prepared without carrying out stirring with use of the electromagnetic stirring devices 50A and 50B (a strand of SUH409L will be referred to as a comparative example strand 1, and a strand of SUS439 will be referred to as a comparative example strand 2).

An X-ray transmission method was carried out with respect to each of the example strands 1 and 2 and the comparative example strands 1 and 2 so as to count the number of surface defects (defects formed by capture of air bubbles or inclusions into a solidified cell) present within 10 mm from a surface layer. In this evaluation, the number of surface defects having a diameter of not less than 0.4 mm was counted. The following Table 1 shows results of counting. Note that Table 1 shows the number of defects per cubic centimeter.

**[Table 1]**

| |
|---|
| Kind of Steel Defect Density (number/cm3) |
| SUH409L Comparative Example Strand 1 0.0029 |
| SUH409L Example Strand 1 0.0000 |
| SUS439 Comparative Example Strand 2 0.0024 |
| SUS439 Example Strand 2 0.0007 |

As shown in Table 1, in the example strands 1 and 2, it was possible to remarkably suppress formation of a surface defect, as compared with the comparative example strands 1 and 2. This appears to be because, since each of the strand examples 1 and 2 was cast in a state where (i) the substantially whole amount of the molten steel discharged through each discharge hole 41A directly reached the surface S and (ii) the molten steel was included in the stirring region, formed by the electromagnetic stirring devices 50A and 50B, until the molten steel reached the surface S from when the molten steel was discharged through the each discharge hole 41A, it was possible to more effectively carry out stirring of the molten steel.

Each of the example strands 1 and 2 and the comparative example strands 1 and 2 thus prepared was subjected to steps (hot rolling, annealing, acid pickling, cool rolling, annealing, and acid pickling) for producing a typical ferrite-based stainless steel sheet, so that a plurality of cold-rolled annealed steel sheets, each having a thickness of 1 mm, were produced. A surface of each steel sheet thus produced was inspected, and it was determined whether the each steel sheet had a quality as a product. As a result, although surfaces of slabs were ground, a few percent (3.9% in a case of SUH409L, and 2.2% in a case of SUS439) in steel sheets prepared with use of the comparative example strands 1 and 2 did not have a quality as a product. In contrast, all of steel sheets prepared with use of the strand examples 1 and 2 had a quality as a product, although surfaces of slabs were not ground.

### Example 2

The following description will discuss another Example of the present invention.

In Example 2, continuous casting of SUS304 was carried out under the following conditions.

### (Continuous casting conditions)

A discharge angle ϕ of each discharge hole 41B: 5°

A width, in a vertical direction, of each discharge hole 41B: 50 mm

A distance L, in the vertical direction, between a surface S and a center of each discharge hole 41B: 220 mm

A distance W between short-side molds 12A and 12B: 1038 mm

A casting speed: 1.40 m/min

A discharge velocity: 932 mm/s

A thickness of a strand: 200 mm

A magnetic flux density at a location 15 mm apart, in a thickness direction, from each of long-side surfaces 11Aa and 11Ba: 1150 G

The above conditions are conditions under which, in a case where stirring is carried out with use of electromagnetic stirring devices 50A and 50B, (i) a substantially whole amount of molten steel discharged through each discharge hole 41B directly reaches short-side surface 12Aa or 12Ba of a mold 10 and (ii) the molten steel is included in a stirring region, formed by the electromagnetic stirring devices 50A and 50B, until the molten steel reaches the short-side surface 12Aa or 12Ba of the mold 10 from when the molten steel is discharged through the each discharge hole 41B.

In Example 2, evaluation was carried out with respect to (i) an example strand 3 prepared while stirring was carried out with use of the electromagnetic stirring devices 50A and 50B and (ii) a comparative example strand 3 prepared without carrying out stirring with use of the electromagnetic stirring devices 50A and 50B. Note that the strand example 3 was prepared by carrying out stirring with use of the electromagnetic stirring devices 50A and 50B from when 900 mm of the strand was drawn out from the mold 10.

Radiographic inspection was carried out with respect to each of the example strand 3 and the comparative example strand 3 so as to count the number of macro-streak-flaws (cracks caused in a case where a mold powder is incorporated into a solidified shell) present at locations 2 mm and 3 mm below a surface layer. The counting was carried out with respect to a middle part of an upper surface of each strand, at locations 800 mm, 1000 mm, 1200 mm, 1500 mm, 2000 mm, 2500 mm, and 3000 mm apart from a casting starting location at which casting was started. In this evaluation, the number of macro-streak-flaws having a diameter of not less than 0.15 mm was counted. Fig. 6 shows results of counting. Fig. 6 shows the numbers of macro-streak-flaws per square millimeter on each of the example strand 3 and the comparative example strand 3. (a) of Fig. 6 is a graph showing the numbers of macro-streak-flaws present at the location 2 mm below the surface layer. (b) of Fig. 6 is a graph showing the numbers of macro-streak-flaws present at the location 3 mm below the surface layer.

As shown in (a) and (b) of Fig. 6, the numbers of macro-streak-flaw present at the locations 2 mm and 3 mm blow the surface layer of the example strand 3 were smaller than those in the comparative example strand 3. This appears to be because, since the strand example 3 was cast in a state where (i) the substantially whole amount of the molten steel discharged through each discharge hole 41B directly reached the short-side surface 12Aa or 12Ba of the mold 10 and (ii) the molten steel was included in the stirring region, formed by the electromagnetic stirring devices 50A and 50B, until the molten steel reached the short-side surface 12Aa or 12Ba from when the molten steel was discharged through the each discharge hole 41B, it was possible to more effectively carry out stirring of the molten steel. In particular, the numbers of macro-streak-flaws were conventionally large at the locations 1000 mm to 2000 mm apart from the casting starting location, as in the comparative example strand 3. In contrast, in the example strand 3, it was possible to reduce the numbers of macro-streak-flaws also at the locations 1000 mm to 2000 mm apart from the casting starting location. From those results, it was found that it was possible to increase yields in grinding of a prepared strand from 96.8% to 97.5%.

### Example 3

The following description will discuss still another Example of the present invention.

In Example 3, continuous casting of SUS304 was carried out under the following conditions.

A discharge angle α of each discharge hole 41: 5°

A discharge area A of each discharge hole 41: 0.0026 m2

A casting width W: 1260 mm

A casting thickness T: 200 mm

A discharge velocity V: 0.70 m/min

A casting speed Vc: 0.7 m/min to 1.2 m/min

A submergence depth L: 0.25 m

An electric conductivity σ of a secondary conductor: 1/ρ = 1/1.3 (ρ represents a specific electric resistance of SUS304, see "Sutenresuko Binran" (Handbook for Stainless Steel), unit: µΩ-m)

In Example 3, a magnetic flux density B was set to 1150 G and a frequency was set to 2.7 Hz, and then an impulse I was calculated in accordance with the foregoing Expressions 1 through 6. As a result, the following Expression 7 was obtained. $0.4 \times 107 \left(G2/μΩ-m\right) < I < 2.5 \times 107 \left(G2/μΩ-m\right)$

In Example 3 in which the impulse falling within a range represented by Expression 7 was applied to the molten steel, it was possible to form a stirring flow having an excellent effect of cleaning a foreign matter from the molten steel, and possible to effectively suppress capture of a foreign matter, present in the molten steel, into a solidified shell.

### Reference Signs List

1A, 1B Continuous casting device
10 Mold
11Aa, 11Ba Long-side surface (first surface)
12Aa, 12Ba Short-side surface (second surface)
40A, 40B Submerged nozzle
41A, 41B Discharge hole
50A, 50B Electromagnetic stirring device (stirring device)
A3Stirring region
S Surface

## Claims

1. A continuous casting method which is carried out with use of a continuous casting device (1A, 1B), the continuous casting device (1A, 1B) including:
a mold (10) which includes a first surface and a second surface, which intersects the first surface, so as to have a surrounding structure;
a submerged nozzle (40A, 40B) which has a discharge hole (41A, 41B) through which molten steel is discharged; and
a stirring device (50A, 50B) which forms a stirring region (A3) by stirring the molten steel in the mold (10),
the method comprising:
a discharging step of discharging, through the discharge hole (41A, 41B) located in the mold (10), the molten steel upward with respect to a horizontal direction and in a direction parallel to the first surface; and
a stirring step of stirring the molten steel so that the stirring region (A3) includes a whole line segment via which the discharge hole (41A, 41B) and a reached location are connected to each other, the reached location being a location on a surface (S) of the molten steel in the mold (10) or on the second surface which location is reached by the molten steel in a case where the molten steel discharged in the discharging step proceeds straight;
wherein, an angle formed by the discharge direction (60, 70) of each of the two discharge holes (41A, 41B) and the horizontal plane is referred to as a discharge angle (Θ, Ø) and is not more than 30°, and a distance between a center of each of the two discharge holes (41A, 41B) and the surface (S) of the molten steel is not less than 180 mm and not more than 230 mm, **characterised in that**, a velocity of a discharge flow is 300-1150 mm/s. .

2. The method as set forth in claim 1, wherein a flow velocity of the molten steel in the stirring region (A3) falls within a range of 0.20 m/s to 0.40 m/s.

3. The method as set forth in claim 1 or 2, wherein the reached location is the location on the surface(S).

4. The method as set forth in any one of claims 1 through 3, wherein an impulse which the molten steel, discharged from the submerged nozzle (40A, 40B), receives by a time when the molten steel reaches the surface (S) is 0.4 × 10⁷ G²/µΩ-m to 2.5 × 10⁷ G²/µΩ-m,
the impulse being calculated according to expressions 1 through 6 below: $\left(A\times 2\right) \times V = W \times T \times Vc$ a discharge velocity V is determined in accordance with the following Expression $V = W \times T \times Vc/2A$ a velocity Vy, in a vertical direction, of the molten steel discharged through the discharge hole (41A, 41B) is obtained in accordance with the following Expression $Vy = V \times sina = W \times T \times Vc \times sina/2A$ time t it takes for the molten steel to reach the surface S from the discharge hole (41A, 41B) (surface reaching time t) is obtained in the accordance with the following Expression $t = L / Vy = L \times W \times T \times Vc \times sina / 2 A$ stirring hydraulic power H applied to the molten steel is obtained in accordance with the following Expression $H = {B}^{2} \times f \times s$ an impulse I which the molten steel, discharged through the discharge hole (41A, 41B), receives by the time when the molten steel reaches the surface S is obtained in accordance with the following Expression $I = H \times t = {B}^{2} \times f \times s \times L \times W \times T \times Vc \times sina / 2 A$ where
a: a discharge angle of a discharge hole (41A, 41B) [°];
A: a discharge area of the discharge hole (41A, 41B) [m²];
W: a casting width [m] (horizontal distance between short-side surfaces (12Aa, 12Ba));
T: a casting thickness [m] (horizontal distance between long-side surfaces (11Aa, 11Ba));
V: a discharge velocity at which molten steel is discharged through the discharge hole (41A, 41B) [m/s];
Vc: a casting speed [m/s];
L: a submergence depth to which a submerged nozzle (40A, 40B) is submerged [m];
B: a magnetic flux density at a location in the molten steel, which location is 15mm apart, in a horizontal direction, from each of the long-side surfaces (11Aa, 11Ba) [G];
f: a frequency of an electromagnetic stirring device (50A, 50B) [Hz];
s: an electric conductivity of a secondary conductor (the molten steel at 1500°C) [1/mW-m].
Vy: a discharge velocity in a vertical direction at which molten steel is discharged through the discharge hole (41A, 41B) [m/s]
t: time it takes for the molten steel to reach the surface S from the discharge hole (41A, 41B) [s]
H: stirring hydraulic power
I: an impulse [G²/µΩ-m]

## Patentansprüche

1. Stranggießverfahren, das unter Verwendung einer Stranggießvorrichtung (1A, 1B) durchgeführt wird, wobei die Stranggießvorrichtung (1A, 1B) Folgendes einschließt:
eine Form (10), die eine erste Oberfläche und eine zweite Oberfläche einschließt, die die erste Oberfläche schneidet, so dass sie eine umgebende Struktur aufweist;
eine Tauchdüse (40A, 40B), die eine Auslassöffnung (41A, 41B) aufweist, durch die Stahlschmelze ausgelassen wird; und
eine Rührvorrichtung (50A, 50B), die eine Rührregion (A3) durch Rühren der Stahlschmelze in der Form (10) bildet, wobei das Verfahren Folgendes umfasst:
einen Auslassschritt des Auslassens der Stahlschmelze durch die Auslassöffnung (41A, 41B), die sich in der Form (10) befindet, nach oben in Bezug auf eine horizontale Richtung und in einer Richtung parallel zu der ersten Oberfläche; und
einen Rührschritt des Rührens der Stahlschmelze, so dass die Rührregion (A3) ein ganzes Liniensegment einschließt, über das die Auslassöffnung (41A, 41B) und eine erreichte Stelle miteinander verbunden sind, wobei die erreichte Stelle eine Stelle auf einer Oberfläche (S) der Stahlschmelze in der Form (10) oder auf der zweiten Oberfläche ist, die von der Stahlschmelze in dem Fall erreicht wird, in dem die Stahlschmelze, die in dem Auslassschritt ausgelassen wird, gerade verläuft;
wobei ein Winkel, der durch die Auslassrichtung (60, 70) jeder der beiden Auslassöffnungen (41A, 41B) und die horizontale Ebene gebildet wird, als Auslasswinkel (Θ, Ø) bezeichnet wird und nicht mehr als 30° beträgt, und ein Abstand zwischen einer Mitte jeder der beiden Auslassöffnungen (41A, 41B) und der Oberfläche (S) der Stahlschmelze nicht weniger als 180 mm und nicht mehr als 230 mm beträgt, **dadurch gekennzeichnet, dass** eine Geschwindigkeit eines Auslassstroms 300-1150 mm/s beträgt.

2. Verfahren gemäß Anspruch 1, wobei eine Strömungsgeschwindigkeit der Stahlschmelze in der Rührregion (A3) innerhalb eines Bereichs von 0,20 m/s bis 0,40 m/s liegt.

3. Verfahren gemäß 1 oder 2, wobei die erreichte Stelle die Stelle auf der Oberfläche (S) ist.

4. Verfahren gemäß einem der Ansprüche 1 bis 3, wobei ein Impuls, den die Stahlschmelze, die aus der Tauchdüse (40A, 40B) ausgelassen wird, zu einem Zeitpunkt erhält, zu dem die Stahlschmelze die Oberfläche (S) erreicht, 0,4 × 10⁷G²/µΩ-m bis 2,5 × 10⁷ G²/µΩ-m beträgt,
wobei der Impuls nach den folgenden Ausdrücken 1 bis 6 berechnet wird: $\left(A\times 2\right) \times V = W \times T \times Vc$ eine Auslassgeschwindigkeit V wird nach dem folgenden Ausdruck bestimmt $V = W \times T \times Vc / 2 A$ eine Geschwindigkeit Vy in vertikaler Richtung der Stahlschmelze, die durch die Auslassöffnung (41A, 41B) ausgelassen wird, wird nach dem folgenden Ausdruck gewonnen $Vy = V \times sina = W \times T \times Vc \times sina / 2 A$ die Zeit t, die die Stahlschmelze benötigt, um die Oberfläche S von der Auslassöffnung (41A, 41B) aus zu erreichen (Oberflächenerreichungszeit t), wird nach dem folgenden Ausdruck gewonnen $t = L / Vy = L \times W \times T \times Vc \times sina / 2 A$ die hydraulische Rührleistung H, die auf die Stahlschmelze angelegt wird, wird nach dem folgenden Ausdruck gewonnen $H = {B}^{2} \times f \times s$ ein Impuls I, den die Stahlschmelze, die durch die Auslassöffnung (41A, 41B) ausgelassen wird, zu dem Zeitpunkt erhält, zu dem die Stahlschmelze die Oberfläche S erreicht, wird nach dem folgenden Ausdruck gewonnen $I = H \times t = {B}^{2} \times f \times s \times L \times W \times T \times Vc \times sina / 2 A$ wobei
a: ein Auslasswinkel einer Auslassöffnung (41A, 41B) [°];
A: eine Auslassfläche der Auslassöffnung (41A, 41B) [m²];
W: eine Gussbreite [m] (horizontaler Abstand zwischen den kurzseitigen Flächen (12Aa, 12Ba));
T: eine Gussdicke [m] (horizontaler Abstand zwischen den längsseitigen Flächen (11Aa, 11Ba));
V: eine Auslassgeschwindigkeit, mit der die Stahlschmelze durch die Auslassöffnung (41A, 41B) ausgelassen wird [m/s];
Vc: eine Gießgeschwindigkeit [m/s];
L: eine Eintauchtiefe, bis zu der eine Tauchdüse (40A, 40B) eingetaucht ist [m];
B: eine magnetische Flussdichte an einer Stelle in der Stahlschmelze, die in horizontaler Richtung 15 mm von jeder der längsseitigen Flächen (11Aa, 11Ba) entfernt ist [G];
f: eine Frequenz einer elektromagnetischen Rührvorrichtung (50A, 50B) [Hz];
s: eine elektrische Leitfähigkeit eines sekundären Leiters (die Stahlschmelze bei 1500 °C) [1/mW-m].
Vy: eine Auslassgeschwindigkeit in vertikaler Richtung, mit der die Stahlschmelze durch die Auslassöffnung (41A, 41B) ausgelassen wird [m/s]
t: Zeit, die die Stahlschmelze benötigt, um die Oberfläche S von der Auslassöffnung (41A, 41B) aus zu erreichen [s]
H: hydraulische Rührleistung
I: ein Impuls [G²/µΩ-m]

## Revendications

1. Procédé de coulée continue qui est réalisé en utilisant un dispositif de coulée continue (1A, 1B), le dispositif de coulée continue (1A, 1B) comprenant :
un moule (10) qui comprend une première surface et une seconde surface, qui croise la première surface, de manière à avoir une structure environnante ;
une buse immergée (40A, 40B) qui a un trou de décharge (41A, 41B) à travers lequel l'acier fondu est déchargé ; et
un dispositif d'agitation (50A, 50B) qui forme une région d'agitation (A3) en agitant l'acier fondu dans le moule (10), le procédé comprenant :
une étape de décharge consistant à décharger, à travers le trou de décharge (41A, 41B) situé dans le moule (10), l'acier fondu vers le haut par rapport à une direction horizontale et dans une direction parallèle à la première surface ; et
une étape d'agitation consistant à agiter l'acier fondu de sorte que la région d'agitation (A3) comprenne un segment de ligne entier par l'intermédiaire duquel le trou de décharge (41A, 41B) et un emplacement atteint sont reliés l'un à l'autre, l'emplacement atteint étant un emplacement sur une surface (S) de l'acier fondu dans le moule (10) ou sur la seconde surface, emplacement qui est atteint par l'acier fondu dans un cas où l'acier fondu déchargé dans l'étape de décharge se déplace en ligne droite ;
dans lequel, un angle formé par la direction de décharge (60, 70) de chacun des deux trous de décharge (41A, 41B) et le plan horizontal est appelé angle de décharge (Θ, Ø) et n'est pas supérieur à 30°, et une distance entre un centre de chacun des deux trous de décharge (41A, 41B) et la surface (S) de l'acier fondu n'est pas inférieure à 180 mm et n'est pas supérieure à 230 mm, **caractérisé en ce que**, une vitesse d'un écoulement de décharge est de 300-1150 mm/s.

2. Procédé selon la revendication 1, dans lequel une vitesse d'écoulement de l'acier fondu dans la région d'agitation (A3) se situe dans une plage de 0,20 m/s à 0,40 m/s.

3. Procédé tel que défini dans la revendication 1 ou 2, dans lequel l'emplacement atteint est l'emplacement sur la surface (S).

4. Procédé tel que défini dans l'une quelconque des revendications 1 à 3, dans lequel une impulsion que l'acier fondu, déchargé par la buse immergée (40A, 40B), reçoit à un moment où l'acier fondu atteint la surface (S) est de 0,4 × 10⁷G2/µΩ-m à 2,5 × 10⁷ G²/µΩ-m,
l'impulsion étant calculée selon les expressions 1 à 6 ci-dessous : $\left(A\times 2\right) \times V = W \times T \times Vc$ une vitesse de décharge V est déterminée selon l'expression suivante $V = W \times T \times Vc / 2 A$ la vitesse Vy, dans une direction verticale, de l'acier fondu déchargé par le trou de décharge (41A, 41B) est obtenue selon l'expression suivante $Vy = V \times sina = W \times T \times Vc \times sina / 2 A$ le temps t que met l'acier fondu pour atteindre la surface S à partir du trou de décharge (41A, 41B) (temps d'atteinte de la surface t) est obtenu selon l'expression suivante $t = L / Vy = L \times W \times T \times Vc \times sina / 2 A$ La puissance hydraulique d'agitation H appliquée à l'acier fondu est obtenue selon l'expression suivante $H = {B}^{2} \times f \times s$ l'impulsion I que reçoit l'acier en fusion, déchargé par le trou de décharge (41A, 41B), au moment où l'acier en fusion atteint la surface S est obtenue selon l'expression suivante $I = H \times t = {B}^{2} \times f \times s \times L \times W \times T \times Vc \times sina / 2 A$ où
a : angle de décharge d'un trou de décharge (41A, 41B) [°] ;
A : surface de décharge du trou de décharge (41A, 41B) [m²] ;
W : largeur de la pièce [m] (distance horizontale entre les surfaces des petits côtés (12Aa, 12Ba)) ;
T : épaisseur de la pièce [m] (distance horizontale entre les surfaces des côtés longs (11Aa, 11Ba)) ;
V : vitesse de décharge à laquelle l'acier fondu est déchargé par le trou de décharge (41A, 41B) [m/s] ;
Vc : vitesse de coulée [m/s] ;
L : une profondeur d'immersion à laquelle une buse immergée (40A, 40B) est immergée [m] ;
B : une densité de flux magnétique à un emplacement dans l'acier fondu, lequel emplacement est distant de 15 mm, dans une direction horizontale, de chacune des surfaces du côté long (11Aa, 11Ba) [G] ;
f : une fréquence d'un dispositif d'agitation électromagnétique (50A, 50B) [Hz] ;
s : conductivité électrique d'un conducteur secondaire (l'acier fondu à 1500°C) [1/mW-m].
Vy : vitesse de décharge dans une direction verticale à laquelle l'acier fondu est déchargé par le trou de décharge (41A, 41B) [m/s].
t : temps nécessaire à l'acier fondu pour atteindre la surface S à partir du trou de décharge (41A, 41B) [s].
H : puissance hydraulique d'agitation
I : une impulsion [G²/µΩ-m]
